

## 1

3,177,073

 HIGH STRENGTH ALUMINUM ALLOY FOR  
PELLET EXTRUSION AND PRODUCT

George S. Foerster, Midland, Mich., assignor to The Dow Chemical Company, Midland, Mich., a corporation of Delaware  
No Drawing. Filed Mar. 26, 1962, Ser. No. 182,648  
2 Claims. (Cl. 75—147)

This invention relates to aluminum alloys and more particularly is concerned with a novel aluminum alloy having particular utility in the preparation of high strength pellet extrusions, to the extruded product and to the process for preparing the product.

In general, this novel aluminum base alloy contains on a weight basis from about 0.5 to about 2.0 percent magnesium, from about 0.5 to about 10 percent silicon, from about 0.5 to about 10 percent of an additive metal, balance aluminum, wherein the silicon and additive metal are maintained within a predetermined ratio and the silicon content is at least equal to or in excess of that needed for formation of magnesium silicide ( $Mg_2Si$ ).

Iron and chromium are employed as the additive metals in this alloy. Chromium is especially preferred as additive since this does not lower the excellent corrosion resistance generally inherent in aluminum base alloys containing magnesium and silicon. The actual amount of additive to be employed in the alloy is varied in accordance with the properties and characteristics, e.g. density, etc., desired in the extruded product. The actual silicon content employed in the alloy, within the range of from 0.5 to 10 percent as set forth hereinbefore, is established in accordance with the equation:

Wt. percent Si =

$$\frac{\text{Wt. percent Mg}}{1.73} + K \text{ (weight percent additive member)}$$

Minimum K values to be used with the additives to assure the incorporation of the desired amount of silicon into the alloy are 0.5 for chromium and 0.2 for iron. Preferably for optimum alloy properties the minimum silicon content is determined using the following K values in the equation; chromium (1.1) and iron (0.5).

The operable concentration range and preferred concentration range of these same additive metals in the alloy are shown in Table I.

TABLE I

| Metal    | Concentration in Alloy<br>(Weight Percent) |                    |
|----------|--------------------------------------------|--------------------|
|          | Operable<br>Range                          | Preferred<br>Range |
| Chromium | 0.5-6                                      | 1.5-3              |
| Iron     | 0.5-8                                      | 3-6                |

The additive members can be used alone in the alloy or a mixture of additives can be employed. With mixtures of additive metals, the concentration of each of the individual members used therein is proportionally reduced so that the total concentration of the additive in the alloy falls within the range and in accordance with the relationship set forth hereinbefore.

The alloy is prepared using foundry alloying and melt techniques as practiced in the aluminum art.

This alloy particularly is suitable for fabricating high strength pellet extrusions. In this operation, a melt of the alloy is prepared and rapidly solidified as by atomizing into pellets. Conveniently the pellets can be produced

## 2

by jet atomizing or wheel atomizing either in an inert atmosphere such as natural gas, nitrogen, argon, etc. for example, or in air. The atomized pellets are fabricated into high strength extrusions using normal pellet extrusion techniques and apparatus.

In this process, because of the rapid cooling of the small pellets the dispersed second phase is present in the alloy in much finer form than in a massive ingot which has a relatively slow cooling rate. Therefore, high strength fabrications exhibiting satisfactory elongation, i.e. ductility in the final product can be extruded using these alloys having the metal ratios and concentrations set forth herein.

For use in the pellet extrusion process, ordinarily the pellets are preheated to a temperature at least that of the extruder container and the heated pellets then are loaded into the container and extruded. However, if desired, the pellets can be used in the extrusion process without preheating. Also the pellets can be precompacted prior to extrusion. By precompacting the pellets under reduced pressure, blistering and formation of internal voids substantially are avoided during any post extrusion heat treatment that may be employed.

The so-extruded product can be solution heat treated, quenched and aged, if desired. In this treatment, preferably the length of time for solution heat treatment is minimized to avoid (1) agglomeration of any dispersed phase that might be present in the alloy, (2) recovery, (3) recrystallization and (4) loss of strength.

For those alloys which contain silicon in excess of the solid solubility of this element in the alloy, high strength extrusions and particularly pellet extrusions unexpectedly can be produced at relatively low extrusion temperatures, i.e. from about 750 to about 850° F. Further increase in the strength of the extrusion results by directly quenching the extruded product as it emerges from the die and subsequently aging.

The following example will serve to illustrate further the utility of the present invention but is not meant to limit it thereto.

## Example I

An aluminum base-magnesium-silicon alloy containing chromium or iron as an additive member was prepared. The alloy was atomized into pellet form. The pellets had a mesh distribution of about 85%—20 +200 (U.S. Standard Sieve) the balance passing through the 200 mesh sieve.

A batch of the atomized pellets was preheated to about 700° F. and placed in the pellet container of a ram extruder which container also was about this same temperature.

The pellets were extruded at an extrusion temperature of about 800° F. and an extrusion rate of about 5 feet per minute into a strip 0.2 inch thick by 1 inch wide. The resulting strip then was solution heat treated at about 970° F. for 1/2 hour, quenched and aged 16 hours at 320° F.

As a control, an alloy containing predetermined amounts of magnesium and silicon without any additive metal was prepared and cast both into ingot and pellet form, extruded and similarly heat treated. A further control was established by adding predetermined quantities of the additive metals to the magnesium-silicon containing alloy and again extruding similar strips from a 3-inch diameter ingot of the alloy. The control extrusions subsequently were heat treated as described hereinbefore.

Standard test bars were prepared and the percent elongation, tensile yield strength and tensile strength of the alloys determined at room temperature. The results of these tests are presented in Table II which follows.

TABLE II

| Run No. | Percent by wt. |     | Other | K    | Test Results |                  |                 | Extrusion Form | Remarks                           |
|---------|----------------|-----|-------|------|--------------|------------------|-----------------|----------------|-----------------------------------|
|         | Mg             | Si  |       |      | E, percent   | TYs, 1000 p.s.i. | TS, 1000 p.s.i. |                |                                   |
| 1       | 1.2            | 0.7 |       |      | 14           | 35               | 40              | I+P            | Control—No additive.              |
| 2       | 1.2            | 0.7 | 2 Cr  |      | 4            | 36               | 40              | I              | Control.                          |
| 3       | 1.0            | 1.0 | 2 Cr  | 0.2  | 13           | 28               |                 | P              |                                   |
| 4       | 1.9            | 2.4 | 2 Cr  | 0.65 | 6            | 46               | 52              | P              | Mn/Cr ratio in inoperative range. |
| 5       | 1.5            | 3.5 | 2 Cr  | 1.3  | 10           | 52               | 59              | P              |                                   |
| 6       | 1.2            | 0.7 | 2 Fe  |      | 10           | 35               | 40              | I              | Control.                          |
| 7       | 1.2            | 0.8 | 6 Fe  | 0.02 | 12           | 26               | 41              | P              |                                   |
| 8       | 1.2            | 2.0 | 6 Fe  | 0.2  | 4            | 41               | 50              | P              | Mn/Fe ratio in inoperative range. |
| 9       | 1.2            | 4.0 | 6 Fe  | 0.55 | 4            | 55               | 62              | P              |                                   |

I=Ingot, P=Pellet.

These results clearly show the unexpected, pronounced increase in strength obtained from pellet extrusions prepared from alloys having a composition in accordance with that set forth hereinbefore as well as demonstrates the need for maintaining the additive metal/silicon ratio within the range prescribed herein.

Various modifications can be made in the present invention without departing from the spirit or scope thereof for it is understood that I limit myself only as defined in the appended claims.

I claim:

1. An aluminum alloy consisting essentially of from about 0.5 to about 2.0 weight percent magnesium, from about 0.5 to about 10 weight percent silicon, an additive metal, balance aluminum, said additive metal being a member selected from the group consisting of chromium and iron and the concentration in weight percent of said additive metal in said alloy being from about 1.5 to about 3 for chromium and from about 3 to about 6 for iron, the weight percent of silicon in said alloy being predetermined within the range of from about 0.5 to about 10 percent in accordance with the equation

Wt. percent Si=

$$\frac{\text{wt. percent Mg}}{1.73} + K \text{ (wt. percent additive metal)}$$

where K is 1.1 for chromium and 0.5 for iron.

2. A high strength aluminum alloy pellet extrusion formed from a pelletized aluminum alloy consisting essentially of from 0.5 to about 2 weight percent magnesium, from about 0.5 to about 10 weight percent silicon, an additive metal, and remainder aluminum, said ad-

ditive metal being a member selected from the group consisting of from about 1.5 to about 3 weight percent chromium and from about 3 to about 6 weight percent iron, and the actual weight percent of silicon in said alloy being predetermined in accordance with the relationship:

$$(a) \text{ wt. percent Si} =$$

$$\frac{\text{wt. percent Mg}}{1.73} + 1.1 \text{ (1.5 to 3 wt. percent chromium)}$$

$$(b) \text{ wt. percent Si} =$$

$$\frac{\text{wt. percent Mg}}{1.73} + 0.5 \text{ (3-6 wt. percent iron)}$$

said extrusion being characterized in the extruded, solution heat treated, quenched and aged condition by an unexpectedly high tensile strength.

## References Cited by the Examiner

## UNITED STATES PATENTS

|           |       |               |       |          |
|-----------|-------|---------------|-------|----------|
| 2,053,925 | 9/36  | Stroup        | ----- | 75—147   |
| 2,280,172 | 4/42  | Stroup        | ----- | 75—147   |
| 2,454,312 | 11/48 | Fritzlen      | ----- | 75—147 X |
| 2,966,731 | 1/61  | Towner et al. | ----- | 75—138 X |
| 3,031,299 | 4/62  | Criner        | ----- | 75—148   |

## FOREIGN PATENTS

|         |       |               |
|---------|-------|---------------|
| 357,805 | 10/31 | Great Britain |
| 440,600 | 1/36  | Great Britain |
| 977,514 | 4/51  | France        |

DAVID L. RECK, Primary Examiner.